# EUROPEAN PATENT SPECIFICATION

(11) **EP 1 080 270 B1**
(45) Date of publication and mention of the grant of the patent: **17.11.2004**
(21) Application number: 99945723.7
(22) Date of filing: 08.04.1999
(51) Int. Cl.: D21H 21/54

(54) **A PROCESS FOR THE PRODUCTION OF PAPER**
EIN VERFAHREN ZUR HERSTELLUNG VON PAPIER
PROCEDE DE PRODUCTION DE PAPIER

(30) Priority: 23.04.1998 EP 98850061; 23.04.1998 US 82784 P
(43) Date of publication of application: 07.03.2001
(73) Proprietor: AKZO NOBEL N.V., 6800 SB Arnhem (NL); Eka Chemicals AB, 445 80 Bohus (SE)
(72) Inventor: SIKKAR, Rein, S-448 34 Floda (SE); PERSSON, Michael, S-413 21 Göteborg (SE); NORELL, Maria, S-436 51 Hovas (SE)
(74) Representative: Jönsson, Christer
(86) International application number: PCT/SE1999/000574
(87) International publication number: WO 1999/054551

(56) References cited:
- EP-A- 0 534 656
- WO-A-97/30220
- J.Chem.Soc., Chem. Commun., 1993, pp. 1784-5,Jing Li et al "C60 Fullerol Formation catalysed by Quaternary ammonium Hydroxides" XP002083225 cited in the application
- Colloids and Surfaces, A: Physicochem. Eng. aspects 108 (1996), pp. 113-116, K.Esumi et al "Preparation of hollow carbon-microbeads from water-in-oil emulsion using amphiphilic carbonaceous material" XP002083226 cited in the application

## Description

The present invention relates to a paper production process. In the present application the term "paper production process" is intended to encompass the entire paper production process, i.e. from the defibration of the wood until the paper product is ready to be supplied to the market. The present invention also relates to paper obtainable by said process, whereby "paper" is to be understood to include also board, paperboard, fibreboard, and cardboard, as well as any other similar cellulosic fibre containing product. Furthermore, the invention relates to paper making additives such as drainage and retention agents that may be used in such a process.

The paper making process usually involves the use of various additives in order to control the paper production process as such and/or the properties of the produced paper. Drainage and retention agents are among the most common paper making additives.

A wide variety of drainage and retention agents are known in the art. These additives are included in the papermaking stock in order to facilitate drainage and/or to increase adsorption of fine particles and additives onto the cellulose fibres so that they are retained with the fibres. The drainage and retention agents employed include natural and synthetic organic polymers, particles of inorganic materials and many combinations thereof. Usually, oppositely charged materials are used. Certain microsize particles, namely colloidal silica particles, in combination with cationic starch, such as for example disclosed in EP-B-41,056 is an example of a commonly used drainage and retention agent. The particles act as flocculants, binding the polymer molecules to larger aggregates. EP-A-534,656 discloses a papermaking process involving addition of a mineral filler, a cationic charge-biasing species, an anionic flocculant, and microparticles being of inorganic cationic source of aluminium. Shell-formed carbon allotrope particles are, however, not described therein. WO 97/30220, discloses a process for making filled paper comprising adding an anionic micro particulate material to the cellulosic suspension. The anionic particulate material can be e.g. swelling clays, zeolites and synthetic particulate silica compounds. However, WO 97/30220 does not relate to shell-formed carbon allotrope particles.

A common feature of the drainage and retention agents referred to above is their contents of certain microsize particles, below referred to as microparticles. It would be desirable to be able to provide a paper production process in which other microparticles than those presently known in the art are used as that would provide, at least ceteris panbus, for a bigger supply of microparticles. In a drainage/retention agent it would be desirable to use micropartides that could provide, at least potentially, for better flocculation. Microparticles that could provide for all of this would of course be especially desirable.

Thus, the problem. to be solved by the present invention is to provide a paper production process in which such microparticles are used.

This problem has been solved by the present invention as defined by the appended claims. More specifically the present invention relates to a process for the production of paper comprising cellulosic fibres, in which at least some of the fibres are treated at some part of the process with microparticles comprising shell-formed carbon allotrope particles.

It has been found that the particle charge density of these microparticles may greatly influence the effect of the drainage/retention agents. It would seem that microparticles having a high particle charge density provide for a potentially better flocculation in a drainage/retention operation. The reason for this is as follows:

In a drainage/retention operation, a cationic polymer and anionic microparticles form complex agglomerates in the stock, which agglomerates are bound together by the anionic microparticles, and the cationic polymer becomes associated with filler material having a more or less anionic surface. The cationic polymer also becomes associated with the cellulosic fibres and fines, both of which are anionic. Upon bonding, the association between the agglomerates and the cellulosic fibres provides flocculation. It would seem that a higher particle charge density of the anionic microparticles would provide for more anionic groups on the particle surface, in turn providing more bond sites and, as a consequence, potentially bigger agglomerate.

In the present application the term "microparticle" indicates a particle having a particle size of up to about 10 µm, preferably up to about 100 nm, and most preferably up to about 20 nm.

The microparticles used in the present invention comprise shell-formed carbon allotrope particles, which may mean that each microparticle consists of one or more shell-formed carbon allotrope particles, but may just as well mean that the microparticles are only partly made up of shell-formed carbon allotrope particles whereas the other part is made up of some other substance.

By "shell-formed carbon allotrope" is meant any carbon allotrope in which the atoms are arranged so as to form a shell, preferably a closed shell having an essentially spherical form. An open shell form, such as for instance the form of a tube with one or more openings, is however not excluded.

In an preferred embodiment of the present invention the shell form is defined by the atomic lattice, i.e. each unit of this lattice constitutes an individual shell. An illustrative and preferred example of this embodiment is of course the fullerene allotrope, e.g. a [60]fullerene or a [70]fullerene. It is however not ruled out that the shell-formed particles may be a so-called "hollow carbon microbeads" as disclosed by K. Esumi et al in Colloids and Surfaces, A: Physicochem. Eng. Aspects 108 (1996) 113-116, in which the shell form is defined by a plurality of atomic lattice units.

In one embodiment, the shell-formed carbon allotrope comprises one or more heteroatom, such as for instance a Si, B, N, S, or P atom. In a particular example, the carbon allotrope is a heterofullerene such as described in "The Chemistry of the Fullerenes" by A. Hirsch, (Georg Thime Verlag, Stuttgart, New York 1994, chapter 9.4.2, page 196).

The carbon allotrope particles may be furnished with addends and/or substituents; the particles may for instance be hydroxylated, sulphonated, or carboxylated. For instance, carbon allotrope particles may be polyhydroxylated fullerene derivatives, so-called fullerols, e.g. prepared according to the methods described by Jing Li et al in J. Chem. Soc., Chem. Commun., 1993, pp 1784-5 ("C₆₀ Fullerol Formation catalysed by Quartenary Ammonium Hydroxides"), or EP 540 311.

The invention can be used in a variety of flocculation operations, including for instance sludge dewatering, waste water treatment, wine clarification; this listing of flocculation operations is of course not exhaustive.

In one embodiment the particles are used for the purpose of improving the dewatering/retention performance of a paper making process, whereby the microparticles are preferably combined with a polymer. The particles and the polymer are added, either mixed or separated from each other, either simultaneously or consecutively, to the papermaking stock, whereby the shell-formed carbon allotrope particles are at least partially hydrophilic, and preferably soluble in aqueous solutions. In this embodiment the carbon allotrope is preferably an anionic fullerene derivative, e.g. a hydroxylated, sulphonated, or carboxylated fullerene derivative. When used for dewatering/retention performance improvement, the carbon allotrope particles are preferably associated with each other, e.g. by means of covalent bonds, electrostatic bonds, ionic bonds, or any similar kind of bonds. The bonds may for instance be constituted by means of one and more hydrocarbyl groups and/or one or more atoms chosen among N, O, P, S, B, and Si. Said atoms may farm an integrated part of the particles or be comprised in an addend or substituent to the particles, but may also form a bridge between addends or substituents of two or more allotrope particles. The hydrocarbyl group may be an addend or substituent common to two or more allotrope particles, but may also form a bridge between addends or substituents of two or more allotrope particles, for instance between atoms chosen among N, O, P, S, B, and Si. The concept of fullerene polymers is discussed in "The Chemistry of the Fullerenes" by A. Hirsch, (Georg Thime Verlag, Stuttgart, New York 1994, chapter 3.2.3, page 64-65), and one way to prepare such fullerene polymers is for instance disclosed in US-A-5,367,051.

The allotrope microparticles may for instance be combined with a polymer having a branched or unbranched hydrocarbon chain, with or without substituents; it may for instance be chosen among starches, chitosans, seed gums such as guar gums, acrylamide-based polymers, poly(diallyldimethyl ammonium chloride), polyethylene imines. polyamines, polyamidoamines, melamine-formaldehyde resins, urea-formaldehyde resins, N-vinylamide-based polymers, or a combination thereof. In one preferred embodiment the polymer has a branched hydrocarbon chain.

Preferably, when used for dewatering/retention purpose, the allotrope microparticles are present in the papermaking stock in an amount of at least 0,005 kg/tonne of pulp, particularly preferred in an amount from about 0,03 to 5 kg/ton of pulp. The unit kg/ton is calculated as dry on dry fibres and optional fillers, and by a "ton" is meant a metric ton.

The present invention also relates to paper obtainable from this dewatering/retention performance improved paper making process.

Furthermore, the present invention relates to a drainage or retention agent comprising at least partially hydrophilic, anionic microparticles comprising shell-formed carbon allotrope particles, which is adapted to be used in said dewatering/retention performance improved paper making process. The partially hydrophilic, anionic microparticles are at least partially made up of carbon allotrope particles that are associated with each other, e.g. by means of covalent bonds, electrostatic bonds, ionic bonds, or any similar kind of bonds. The bonds may for instance be constituted by means of one and more hydrocarbyl groups and/or one or more atoms chosen among N, O, P, S, B, and Si. Said atoms may form an integrated part of the particles or be comprised in an addend or substituent to the particles, but may also form a bridge between addends or substituents of two or more allotrope particles. The hydrocarbyl group may be an addend or substituent common to two or more allotrope particles, but may also form a bridge between addends or substituents of two or more allotrope particles, for instance between atoms chosen among N, O, P, S, B, and Si.

The present invention will now be illustrated by means of some non-limiting examples.

### EXAMPLES

Example 1: Polyhydroxylated fullerene derivatives, so-called fulferols, were prepared essentially according to the method described by Jing Li et al in J. Chem. Soc., Chem. Commun., 1993, pp 1784-5 ("C₆₀ Fullerol Formation catalysed by Quartenary Ammonium Hydroxides"). More particularly, two kinds of fullerols, fullerol A and fullerol B, were produced:

Fullerol A and B were produced according to the following procedure: C-60 Fullerene was mixed with 1,7-diaminoheptane ( molar ratio of 2:1) in benzene. The reagents were stirred at ambient temperature for 48 hours after which the reaction mixture, consisting of coupled aminofullerenes, was subjected to hydroxylation according to the method described by Jing-Li et al in J. Chem. Soc., Chem. Commun., 1993, pp 1784-5 ("C60 Fullerol Formation catalysed by Quartenary Ammonium Hydroxides"). The watersoluble reaction mixture was precipitated by addition of methanol which yielded Fullerol A as a brownish solid. The mother liquor was evaporated to dryness and the residue again dissolved in water and precipitated by methanol yielding Fullerol B as an almost black solid. The mass yields of Fullerol A and B were about equal. The two fractions were used in the following examples.

Example 2: In the following tests, drainage performance was evaluated by means of a Dynamic Drainage Analyser (DDA), available from Akribi AB, Sundsvall, Sweden, which measures the time required to drain a set volume of stock through a wire when removing a plug and applying a vacuum to the side of the wire opposite the stock.

The drainage tests were made using a stock having a pH of 8,5 and a consistency of 0,3 %, which contained 70 % cellulosic fibres, 60 % bleached hardwood Kraft and 40 % bleached softwood Kraft and 30 % Hydrocarb 60. The stock further contained 0,3 g/l Na₂SO₄*10 H₂O In test 2A microparticles according to the present invention were tested in conjunction with a cationic polymer, Raisamyl 142, which is a conventional medium-high cationised starch having a degree of substitution of 0.042, which was added to the stock in an amount of 12 kg/ton. In test 2B microparticles according to the present invention were tested in conjunction with a cationic polyacrylamide of 10 mole-% cationic charge and a molecular weight of about 6 million Da, which was added to the stock in an amount of 1 kg/ton.

The stock was stirred in a baffled jar at a speed of 1500 rpm throughout the test and chemical additions to the stock were conducted as follows:
i) adding cationic starch or polymer followed by stirring for 30 seconds,
ii) adding the microparticles comprising shell-formed carbon allotrope particles, followed by stirring for 15 seconds,
iii) draining the stock while automatically recording the drainage time.

Table I shows the drainage results, in seconds, obtained in test 2A when using varying dosages of fullerols A and B; shorter drainage times means better drainage performance of the fullerols. Without addition of microparticles, the stock had a drainage time of 18 seconds.

**Table I**

| Microparticles | 0.25 kg/ton | 0.5 kg/ton | 0.75 kg/ton | 1.0 kg/ton | 1.5 kg/ton | 2.0 kg/ton | 2.5 kg/ton |
|---|---|---|---|---|---|---|---|
| Fullerol A | 15.9 | 12.8 | 11.5 | 9.78 | 8.57 | 6.79 | 6.7 |
| Fullerol B | 16.2 | 14.6 | 13.5 | 12.2 | 9.41 | 8.87 | 10.5 |

Table II shows the drainage results, in seconds, obtained in test 2B when using varying dosages of fullerols A and B. Without addition of microparticles, the stock had a drainage time of 16.9 seconds.

**Table II**

| Microparticles | 0.1 kg/ton | 0.25 kg/ton | 0.5 kg/ton | 0.75 kg/ton | 1.0 kg/ton | 2.0 kg/ton |
|---|---|---|---|---|---|---|
| Fullerol A | 15.6 | 14.3 | 13.1 | 12.8 | 13.6 | - |
| Fullerol B | 16.2 | 15.4 | 15.2 | 15.3 | 15.1 | 15.7 |

As can be seen in Table I as well as in Table II, the microparticles according to the invention had a clear effect on the drainage performance.

Example 3: In these test series, retention was evaluated by means of the DDA used in Example 2 in combination with a nephelometer. First pass retention was evaluated by measuring the turbidity of the filtrate, the white water, obtained by draining the stock. Additives and addition order in test 3A were the same as in test 2A, and the conditions prevailing in test 3B were also applied in test 2B.

Table III shows the retention effect measured in test 3A as turbidity of white water obtained by dosing varying amounts of fullerols A and B, where dosages are in kg/ton. Without addition of microparticles, the stock had a turbidity of 119 NTU.

**Table III**

| Microparticles | 0.5 kg/ton | 0.75 kg/ton | 1.0 kg/ton | 1.5 kg/ton | 2.0 kg/ton | 2.0 kg/ton |
|---|---|---|---|---|---|---|
| Fullerol A | 97 | 89 | 83 | 72 | 75 | 66 |
| Fullerol B | 106 | 102 | 97 | 73 | 76 | 86 |

Table IV shows the retention effect measured in test 3B as turbidity of white water obtained by dosing varying amounts of fullerols A and B, where dosages are in kg/ton. Without addition of microparticles, the stock had a turbidity of 96 NTU.

**Table IV**

| Microparticles | 0.1 kg/ton | 0.5 kg/ton | 0.75 kg/ton | 1.0 kg/ton | 2.0 kg/ton |
|---|---|---|---|---|---|
| Fullerol A | 94 | 73 | 71 | 78 | - |
| Fullerol B | 92 | 83 | 85 | 88 | 91 |

As can be seen in Table III as well as in Table IV, the microparticles according to the invention had a clear impact on the retention effect.

## Claims

1. A process for the production of paper comprising cellulosic fibres, in which at least some of the fibres are treated at some part of the process with microparticles,
**characterised in that** the microparticles comprise shell-fermed carbon allotrope particles.

2. A process according to claim 1, **characterised in that** the carbon allotrope is a fullerene and/or a fullerene derivative.

3. A process according to claim 2, **characterised in that** the fullerene is a [60]fullerene or a [70]fullerene.

4. A process according to any preceding claim, **characterised in that** said shell-formed carbon allotrope comprises at least one heteroatom.

5. A process according to any preceding claim, **characterised In that** the carbon allotrope particles are furnished with addends and/or substituents.

6. A process according to claim 1, **characterised in that** said microparticles and a polymer are added to a papermaking stock, and **in that** said shell-formed carbon allotrope particles are at least partially hydrophilic.

7. A process according to claim 6, **characterised in that** said shell-formed carbon allotrope particles are soluble in aqueous solutions.

8. A process according to claim 6, **characterised in that** the carbon allotrope is an anionic fullerene derivative.

9. A process according to claim 6, **characterised in that** the carbon allotrope is a hydroxylated, sulphonated, or carboxylated fullerene derivative.

10. A process according to claim 6, **characterised in that** two or more of the shell-formed carbon allotrope particles are associated with each other.

11. A process according to claim 10, **characterised in that** two or more of the shell-formed carbon allotrope particles are associated with each other by means of at least one hydrocarbyl group and/or at least one atom chosen among N, O, P, S, B, and Si.

12. A process according to claim 10, **characterised in that** the polymer is chosen among starches, chitosans, guar gums, acrylamide-based polymers, poly(diallyldimethyl ammonium chloride), polyethylene imines, polyamines, polyamidoamines, melamine-formaldehyde resins, urea-formaldehyde resins, N-vinylamide-based polymers, or a combination thereof.

13. Paper obtainable from the process according to any one of claims 6-12.

## Patentansprüche

1. Verfahren zur Herstellung von Papier, das Cellulosefasern umfasst, wobei mindestens ein Teil der Fasern in einem Abschnitt des Verfahrens mit Mikroteilchen behandelt wird, **dadurch gekennzeichnet, dass** die Mikroteilchen schalenförmige allotrope Kohlenstoffteilchen umfassen.

2. Verfahren gemäß Anspruch 1, **dadurch gekennzeichnet, dass** der allotrope Kohlenstoff ein Fulleren und/oder ein Fullerenderivat ist.

3. Verfahren gemäß Anspruch 2, **dadurch gekennzeichnet, dass** das Fulleren ein [60]Fulleren oder ein [70]Fulleren ist.

4. Verfahren gemäß einem der vorstehenden Ansprüche, **dadurch gekennzeichnet, dass** der schalenförmige allotrope Kohlenstoff mindestens ein Heteroatom umfasst.

5. Verfahren gemäß einem der vorstehenden Ansprüche, **dadurch gekennzeichnet, dass** die allotropen Kohlenstoffteilchen mit Zusätzen und/oder Substituenten versehen sind.

6. Verfahren gemäß Anspruch 1, **dadurch gekennzeichnet, dass** die Mikroteilchen und ein Polymer einer Stoffmasse zur Papierherstellung zugegeben werden und die schalenförmigen allotropen Kohlenstoffteilchen mindestens teilweise hydrophil sind.

7. Verfahren gemäß Anspruch 6, **dadurch gekennzeichnet, dass** die schalenförmigen allotropen Kohlenstoffteilchen in wässrigen Lösungen löslich sind.

8. Verfahren gemäß Anspruch 6, **dadurch gekennzeichnet, dass** der allotrope Kohlenstoff ein anionisches Fullerenderivat ist.

9. Verfahren gemäß Anspruch 6, **dadurch gekennzeichnet, dass** der allotrope Kohlenstoff ein hydroxyliertes, sulfoniertes oder carboxyliertes Fullerenderivat ist.

10. Verfahren gemäß Anspruch 6, **dadurch gekennzeichnet, dass** zwei oder mehrere der schalenförmigen allotropen Kohlenstoffteilchen miteinander assoziiert sind.

11. Verfahren gemäß Anspruch 10, **dadurch gekennzeichnet, dass** zwei oder mehrere der schalenförmigen allotropen Kohlenstoffteilchen miteinander durch mindestens einen Kohlenwasserstoffrest und/oder mindestens ein aus N, O, P, S, B und Si ausgewähltes Atom assoziiert sind.

12. Verfahren gemäß Anspruch 10, **dadurch gekennzeichnet, dass** das Polymer aus Stärken, Chitosanen, Guargummis, Polymeren auf Acrylamidbasis, Poly(diallyldimethylammoniumchlorid), Polyethyleniminen, Polyaminen, Polyamidoaminen, Melaminformaldehydharzen, Harnstoffformaldehydharzen, Polymeren auf N-Vinylamidbasis oder einer Kombination davon ausgewählt ist.

13. Papier, erhältlich durch das Verfahren nach einem der Ansprüche 6 bis 12.

## Revendications

1. Procédé de production de papier comprenant des fibres cellulosiques, dans lequel au moins certaines de ces fibres sont traitées avec des microparticules en un certain point du procédé, **caractérisé en ce que** ces microparticules comprennent des particules d'une variété allotropique de carbone en forme de coque.

2. Procédé conforme à la revendication 1, **caractérisé en ce que** la variété allotropique de carbone est un fullerène et/ou un dérivé de fullerène.

3. Procédé conforme à la revendication 2, **caractérisé en ce que** le fullerène est un fullerène C₆₀ ou un fullerène C₇₀.

4. Procédé conforme à l'une des revendications précédentes, **caractérisé en ce qu'**il y a, dans ladite variété allotropique de carbone en forme de coque, au moins un hétéroatome.

5. Procédé conforme à l'une des revendications précédentes, **caractérisé en ce que** les particules de variété allotropique de carbone sont munies de fragments ajoutés et/ou de substituants.

6. Procédé conforme à la revendication 1, **caractérisé en ce que** l'on ajoute lesdites microparticules et un polymère à une pâte à papier, et **en ce que** lesdites particules de variété allotropique de carbone en forme de coque sont au moins partiellement hydrophiles.

7. Procédé conforme à la revendication 6, **caractérisé en ce que** lesdites particules de variété allotropique de carbone en forme de coque sont solubles dans des solutions aqueuses.

8. Procédé conforme à la revendication 6, **caractérisé en ce que** la variété allotropique de carbone est un dérivé anionique de fullerène.

9. Procédé conforme à la revendication 6, **caractérisé en ce que** la variété allotropique de carbone est un dérivé hydroxylé, sulfoné ou carboxylé de fullerène.

10. Procédé conforme à la revendication 6, **caractérisé en ce que** des particules de variété allotropique de carbone, au nombre de deux ou plus, sont associées les unes avec les autres.

11. Procédé conforme à la revendication 10, **caractérisé en ce que** des particules de variété allotropique de carbone, au nombre de deux ou plus, sont associées les unes avec les autres au moyen d'au moins un groupe hydrocarbyle et/ou d'au moins un atome choisi parmi les atomes d'azote, d'oxygène, de phosphore, de soufre, de bore et de silicium.

12. Procédé conforme à la revendication 10, **caractérisé en ce que** le polymère est choisi parmi les amidons, les chitosanes, les gommes de guar, les polymères à base d'acrylamide, le poly(chlorure de diallyl-dimé-thyl-ammonium), les polyéthylène-imines, les polyamines, les polyamidoamines, les résines mélamine-formaldéhyde, les résines urée-formaldéhyde et les polymères à base de N-vinyl-amide, ou est une combinaison de tels polymères.

13. Papier qu'on peut obtenir par un procédé conforme à l'une des revendications 6 à 12.
